

## UNITED STATES PATENT OFFICE

2,453,097

SOLUTION CONSISTING OF A POLYMERIC  
N-VINYL PYRROLE COMPOUND AND  
CHLOROFORMMichael T. Ornik, Binghamton, N. Y., assignor  
to General Aniline & Film Corporation, New  
York, N. Y., a corporation of DelawareNo Drawing. Application November 8, 1945,  
Serial No. 627,529

## 4 Claims.

1

This invention relates to the manufacture of sheets, film, or foils composed of polymeric N-vinyl compounds. More particularly, the invention relates to a method of facilitating the removal of such sheets, films, and foils from the surface upon which they are cast.

Polymeric N-vinyl pyrroles of a molecular weight sufficient to produce self-sustaining films and foils, such as polyvinylcarbazole, polyvinylisopropylcarbazole, polyvinyltetrahydrocarbazole, polyvinylindole, polyvinylpropylcarbazole, polyvinylnaphthocarbazole, and the like are described in United States Patent 2,072,465. In the manufacture from such polymers of sheets, foils and films ranging from 0.001 to 0.05 inch in thickness, and of any suitable width, the polymeric N-vinyl pyrrole compound is dissolved in a suitable solvent and a plasticizer added to make the composition which in the parlance of the trade is called a "dope." This dope is cast on the surface of a slowly rotating wheel or drum having a smooth nickel or chrome plated surface, or on the surface of an endless metallic band, and the solvents removed from the deposited material by means of heated air. Finally, the dried or cured material is stripped from the casting surface in the form of a continuous sheet which is wound upon a shaft for storage or further use, such as insulating foil, protective sheeting, and for coating with emulsions to form photographic film. Notwithstanding that the bulk of the solvent has been removed from the film when it reaches the point where it is stripped from the casting surface, difficulty is experienced in the removal of the material from the casting surface.

Regardless of the solvent employed and hereinbefore recommended such as, for example, benzene, toluene, xylene, dioxane, ethylene dichloride, and the like, or mixtures thereof, the cast film or foils adheres so tightly to all known surfaces such as, stainless steel, Monel metal, chrome plate, copper, tin, silver, glass, resin surfaces, and the like, that it requires considerable force to remove it. This causes the film to strip off in an unsteady manner with considerable jerking. Vibrations are thus set up as the result of which the surface of the film or foil develops cross-wise markings, which distinctly impairs the quality of the resulting product. The adhesion is frequently so great as to cause small portions of the film to be torn away from the main body of the material and left upon the casting surface.

In order to obviate the above difficulties, it has been suggested that the casting surface be wetted with water or other wetting solutions, such as

water, benzene, or chloroform. A casting solution containing 50% to 70% casting dope and 50% to 30% chloroform is usually employed. In addition, after the film is cast, it is dried in an oven at 150° F. for 15 to 20 minutes. The film is then stripped from the casting surface and is dried again.

It has been found that the use of chloroform as a casting solvent is not satisfactory because it is difficult to remove the chloroform from the film.

It is an object of the present invention to provide a casting solution which will facilitate the removal of the film from the casting surface.

It is another object of the present invention to provide a casting solution which will facilitate the removal of the film from the casting surface.

It is a further object of the present invention to provide a casting solution which will facilitate the removal of the film from the casting surface.

It is a still further object of the present invention to provide a casting solution which will facilitate the removal of the film from the casting surface.

It is an object of the present invention to avoid the above-mentioned difficulties and to provide a means whereby such films, sheets, or foils may be stripped from a casting surface with ease and without impairment of their quality.

Another object is to provide an improved method of stripping polymeric N-vinyl pyrrole compounds from a casting surface.

These and further objects will become apparent in the following description.

I have discovered that I am enabled to achieve the objects of the present invention by selecting a solvent which not only acts as a plasticizer for

the film-forming, polymeric N-vinyl pyrrole compounds and imparts the aforesaid physical characteristics thereto, but also aids in the stripping of the cast film or foil after drying or curing. This solvent consists of chloroform. Halogenated hydrocarbons in general have been frequently suggested for use as solvents or plasticizers for various resins and polymeric materials. Rather surprisingly, however, chloroform alone of such solvents is capable of imparting plasticity to the

polymeric N-vinyl pyrrole foils and of reducing the interfacial adhesion of such foils to the casting surface, so that the foils may be easily stripped from any one of the known casting surfaces.

Chloroform, used as a single solvent, is preferred. When used as such, it has the combined properties of a solvent, plasticizer, and stripping agent. If it is used as a co-solvent with aromatic compounds or other chlorinated aliphatic compounds either alone or in admixture with an aromatic hydrocarbon, its desirable plasticizing and stripping properties are inhibited. Its use, therefore, alone with polymeric N-vinyl pyrrole compounds leads to a highly efficient and continuous method for casting sheets, films, and foils which is impossible when using other solvents or solvent combinations.

The polymeric N-vinyl pyrrole compounds used herein are, as stated, capable of producing self-sustaining foils and films when cast from a solution of the polymer. Generally, said polymers have a K value ranging from 130 to about 170.

In practicing the present invention, any un-plasticized polymeric N-vinyl pyrrole compound of the type aforesaid may be employed, such as those obtained by the procedure described in the above-

mentioned patent. A solution is prepared by dissolving an appropriate amount of the polymeric N-vinyl pyrrole compound in chloroform. The amount of chloroform employed is in the ratio of 135 to 145 parts by weight to approximately 3 to 8 parts by weight of the polymer. The solution is then filtered by any of the conventional filtration methods to give a clear solution, free of any foreign or undissolved particles. Air, which may be present in the solution, may be removed by vacuum or by heating the solution at 50° C.-60° C. for one hour.

The clear solution of the polymeric N-vinyl pyrrole compound is then fed onto a smooth surfaced drum or endless band by means of a hopper, which is fitted with a micrometer adjustment for foil thickness control.

Drying or curing is accomplished by passing low velocity air at 30° C.-60° C., over the cast solution in a direction counter to that of the moving wheel or band.

For a fuller understanding of the nature and objects of the invention, reference is made to the following examples which are given merely to further illustrate the invention, and they should be regarded as exemplary and not as limitative. All the parts by weight.

*Example I*

A solution or dope is made up as follows:

|                                                 | Parts |
|-------------------------------------------------|-------|
| Polyvinyl carbazole<br>(K=average of about 170) | 4     |
| Chloroform                                      | 143   |

This solution was cast upon the polished periphery of a drum to form a layer which upon drying would produce a film of about 0.008 of an inch in thickness. The partially dried film was removed with ease when taken up by the guide roll leading to the drying chamber.

The advantages of the invention are brought home by contrasting the above procedure with the following, illustrating the effect of adding a co-solvent to a chloroform solution of a polyvinyl carbazole dope from which a film is cast.

|                                              | Parts |
|----------------------------------------------|-------|
| Polyvinyl carbazole<br>(K=average about 170) | 4     |
| Chloroform                                   | 52    |
| Toluene                                      | 91    |

This solution was cast in the manner described above. The partially dried film was removed with difficulty and its surface, which was face to face with the casting surface, showed crosswise markings causing impairment of the film.

The procedure of the above example was repeated with the exception that chloroform was substituted by the same amount of ethylene dichloride. The partially dried foil in this case adhered tenaciously to the casting surface and could not be stripped so as to be placed on the guide roll leading to the drying chamber.

*Example II*

|                                                            | Parts |
|------------------------------------------------------------|-------|
| 5 Polyvinyl isopropylcarbazole<br>(K=average of about 130) | 8     |
| Chloroform                                                 | 138   |

*Example III*

|                                                              | Parts |
|--------------------------------------------------------------|-------|
| 10 Polyvinyl tetrahydrocarbazole<br>(K=average of about 130) | 7.5   |
| Chloroform                                                   | 144   |

The solutions of Examples II and III when cast resulted in very satisfactory films, which were readily removed from the casting surfaces and possessed the same satisfactory properties as the film of Example I.

It is evident that the solutions or dopes prepared in accordance with this invention are not limited for casting on a peripheral surface, but are also capable of being cast on endless metallic belts to give films, foils, or sheets which are cleanly stripped from the casting surface.

While the present invention has been described in considerable detail with reference to preferred procedures and materials, it is to be understood that the invention is not limited thereto and that numerous variations may be made in the procedures herein described. All such modifications and variations are within the scope of the invention as defined by the appended claims.

I claim:

1. A solution, which upon being cast, yields foils and films of polymeric N-vinyl pyrrole compounds of improved stripping properties consisting of 3 to 8 parts by weight of a polymeric N-vinyl pyrrole compound in 135 to 145 parts by weight of chloroform.

2. A solution, which upon being cast, yields foils and films of poly N-vinylcarbazole of improved stripping properties consisting of 4 parts by weight of said polymer dissolved in 143 parts by weight of chloroform.

3. A solution, which upon being cast, yields foils and films of poly N-vinylisopropylcarbazole of improved stripping properties consisting of 8 parts by weight of said polymer dissolved in 138 parts by weight of chloroform.

4. A solution, which upon being cast, yields foils and films of poly N-vinyltetrahydrocarbazole of improved stripping properties consisting of 7.5 parts by weight of said polymer dissolved in 144 parts by weight of chloroform.

MICHAEL T. ORINIK.

**REFERENCES CITED**

The following references are of record in the file of this patent:

**UNITED STATES PATENTS**

| Number    | Name         | Date         |
|-----------|--------------|--------------|
| 2,072,465 | Reppe et al. | Mar. 2, 1937 |